

1

3,425,551  
FLOTATION SEPARATION OF METALLIC  
SULFIDE ORES

Robert E. Baarson, La Grange, and Paul L. Du Brow, Chicago, Ill., assignors, by mesne assignments, to Armour Industrial Chemical Company, a corporation of Delaware  
No Drawing. Filed Aug. 15, 1966, Ser. No. 572,240  
U.S. Cl. 209—166 7 Claims  
Int. Cl. B03d 1/14

ABSTRACT OF THE DISCLOSURE

Dithiocarbonates and di-dithiocarbonates as collectors in froth flotation separation of sulfide minerals from metallic sulfide ores, particularly oxidized metallic sulfide ores.

This invention relates to a process for froth flotation separation of metallic sulfide ores, and more particularly to the use therein of dithiocarbonate compounds as flotation collectors.

In treating crude ores and mineral products to separate the valuable minerals, such as copper, lead and zinc, from the crude material, the process of froth flotation depends for its efficacy on the ability of the collector to wet selectively some constituents of the crude material while other desirable mineral particles of the crude material remain unwetted and adhere to air bubbles which float to the surface of the mixture and are removed as a concentrate in the froth. Coating finely-divided mineral particles is accomplished by agitating a mixture of ore, water and a suitable chemical collector in a conditioner for a short period of time during which the chemical attaches to or associates with the surface of the mineral particles to form a new surface which is more water repellent than the original surface and which is thereby air avid and tends to more easily adhere to air bubbles injected into the system. Sodium ethyl xanthate has been previously used as a collector. Minerals that naturally tend to resist wetting may be treated so that their surfaces will be wetted and they will then sink in the water and not be floated with the concentrates containing desired mineral particles.

An object of this invention is to provide a process in which dithiocarbonate compounds are employed as flotation collectors in the separation of metallic sulfide ores, and particularly oxidized metallic sulfide ores.

Another object is to provide a process in which dithiocarbonate compounds are used in the recovery of copper sulfide.

A further object is to provide a process in which flotation collectors in the nature of dithiocarbonate compounds and their alkali metal salts derived from quaternary ammonium compounds are useful in the flotation treatment of oxidized copper sulfide mineralization.

Other specific objects and advantages will appear as the specification proceeds.

The dithiocarbonates which are useful as collectors in our process have the following structure:



wherein X is a monovalent cation selected from the group consisting of an alkali metal and a quaternary ammonium radical having the structure  $(R_1R_2R_3R_4N)^+$ , each  $R_1$ ,  $R_2$ ,  $R_3$  and  $R_4$  is selected from the group consisting of aliphatic hydrocarbon radicals having from 1 to 22 carbon atoms, provided that at least one and not more than 2 of the  $R_2$ ,  $R_3$  and  $R_4$  radicals contain from 6 to 22 carbon atoms;  $y$  is an integer from 1 to 2; and M is selected from the group consisting of  $R_1$  and  $-(CH_2)_xR_5R_6R_7NOCSS$

2

wherein each  $R_5$ ,  $R_6$  and  $R_7$  is selected from the group consisting of alkyl radicals having from 1 to 3 carbon atoms and  $x$  is an integer from 2 to 4.

The hereinabove described dithiocarbonates may be derived from quaternary ammonium compounds. The dithiocarbonates can also be prepared from quaternized polyalkylene polyamines such as those manufactured by Armour Industrial Chemical Company, a division of Armour and Company, under the trademark Duoquad, or from quaternized imidazolines.

Alkali metal radicals coming within the hereinabove definition of X include sodium, potassium, rubidium and cesium. However we prefer to employ sodium as the alkali metal radical contained in the collectors useful to our process.

Examples of long chain aliphatic hydrocarbon radicals as occurrences of R containing from 6 to 22 carbon atoms within the hereinabove definition of R include hexyl, heptyl, octyl, decyl, dodecyl, tetradecyl, hexadecyl, octadecyl, octadecenyl, octadecadienyl, octadecatrienyl, decosy, eicosyl, and mixtures of the foregoing radicals such as are contained in naturally occurring glycerides such as coconut oil, tallow, soybean oil, and the like. These long chain aliphatic hydrocarbon radicals may be either straight or branched chain, saturated or unsaturated.

Examples of short chain aliphatic hydrocarbon radicals as occurrences of R containing from 1 to 6 carbon atoms within the hereinabove definition of R include methyl, ethyl, propyl, butyl and pentyl. We prefer to employ methyl.

Especially useful collectors which can be utilized in the practice of our process are dithiocarbonates derived from quaternary ammonium compounds with the trademark Arquad, by Armour Industrial Chemical Company, a division of Armour and Company, having the letter designation "C" for the symbol "coco" indicating that the long chain hydrocarbon radicals in the compound are mixtures derived from coconut oil, the letter "S" for the symbol "soya" indicating mixtures derived from soybean oil, and the letter "T" for the symbol "tallow" indicating mixtures derived from tallow.

In deriving the desired dithiocarbonates, the quaternary ammonium hydroxide is reacted with carbon disulfide in the presence of sodium hydroxide to form the

45 sodium salt of dithiocarbonate, for example, N,N,N-trimethyl-N-cocoammonium sodium dithiocarbonate. The dithiocarbonates having a quaternary ammonium cation may be formed by omitting the sodium hydroxide, viz. Di - (N,N,N-trimethyl - N - cocoammonium) dithiocarbonate. In preparing the dithiocarbonates from quaternized polyalkylene polyamines, the di-dithiocarbonate is formed, viz. N,N - dimethyl-N-coco-N',N',N' - trimethyl trimethylene di-ammonium di-(sodium dithiocarbonate).

50 In the practice of the process of this invention, suitable mineral containing sulfide ores may be comminuted to a suitable size for flotation by any of the methods known such as crushing and then grinding in a ball mill. Lime may be added to obtain a pH in the alkaline range. We prefer in the laboratory to grind a 500 gram sample of ore for 2 minutes in a laboratory ball mill at about 55 50% solids in a water suspension and add CaO to obtain a pH of 12.0 to 12.3. The ground ore, water and lime mixture (called a pulp) may be charged directly to a flotation collector such as a Fagergren cell for flotation and the pulp may be further diluted with water. A frother, such as pine oil, and the collector may then be added to the cell and the water suspension of finely-divided metallic sulfide ores is conditioned before the forced introduction of air into the system. We prefer to add frother at about 0.04 #/t. (pounds of chemical per ton of dry ore), collector at a rate of about 0.005 to

0.5 #/t. and an additional increment of about 0.04 #/t. frother after 4 minutes of float time. In synthesizing the collector we prefer to prepare it at various concentrations in isopropyl alcohol or other suitable alcohols as solvents in order to facilitate collector addition to the cell, although the collector may be added in solid form or in a water solution. Flotation may be conducted for from about 3 minutes to about 15 minutes or longer with varying concentrates being collected. We prefer a conditioning time of one minute and flotation for 7 minutes, with only one rougher concentrate containing floated desirable mineral particles being collected.

The above-described process utilizing dithiocarbonate compounds provides exceptional flotation selectivity for copper sulfide mineralization, especially of oxidized copper sulfide ores.

The following specific examples are given to illustrate and to more fully and clearly disclose the present process, but are not to be construed as limiting the scope of our invention:

#### EXAMPLE I

In each test a 500 gram sample of fresh copper sulfide ore analyzing 4.0 to 4.5% Cu was ground in a laboratory ball mill to the approximate size distribution shown in Table I at 50% solids in a water suspension. Lime was added to obtain pH 12.0. The ground ore pulp was transferred to a Fagergren laboratory flotation cell where the ore pulp was conditioned for 1 minute after the addition of the collector and the frother as indicated in Table II. Following conditioning, flotation was conducted for 5 minutes, then an additional increment of 0.04 #/t. of frother was added to the cell, and flotation continued for a total of 9 minutes. Table II shows the collector and frother applied and the reagent addition rates used. Table III shows the metallurgical results obtained.

TABLE I.—SCREEN ANALYSIS—BALL MILL GRIND

| Mesh size fraction | Weight percent | Accumulative weight percent |
|--------------------|----------------|-----------------------------|
| +80.....           | 1.0            | 1.0                         |
| 80-100.....        | 5.2            | 6.2                         |
| 100-150.....       | 14.9           | 21.1                        |
| 150-200.....       | 29.1           | 50.2                        |
| 200-325.....       | 48.4           | 98.6                        |
| -325.....          | 1.4            | 100.0                       |
|                    | 100.0          |                             |

TABLE II

| Test No. | Collector                                                | Collector, #/T | Iso-propanol, #/T | Pine oil, #/T |
|----------|----------------------------------------------------------|----------------|-------------------|---------------|
| 1.....   | Di-(N,N-dimethyl-N,N-dicoco ammonium) dithiocarbonate.   | 0.133          | 0.200             | 0.08          |
| 2.....   | N,N-dimethyl-N,N-dicoco ammonium sodium dithiocarbonate. | 0.074          | 0.222             | 0.08          |
| 3.....   | Di-(N,N,N-trimethyl-N-cocoammonium) dithiocarbonate.     | 0.079          | 0.237             | 0.08          |
| 4.....   | Std. <sup>1</sup>                                        | 0.06           | .....             | 0.08          |

<sup>1</sup>Minerac 27, a xanthogen sulfate.

TABLE III

| Test No. | Analyses, weight percent Cu |       | Distribution, weight percent recovery of Cu in concentrate |
|----------|-----------------------------|-------|------------------------------------------------------------|
|          | Concentrate                 | Tails |                                                            |
| 1.....   | 26.20                       | 0.18  | 96.49                                                      |
| 2.....   | 24.64                       | 0.18  | 96.64                                                      |
| 3.....   | 29.87                       | 0.37  | 92.42                                                      |
| 4.....   | 16.11                       | 0.15  | 97.40                                                      |

#### EXAMPLE II

The test procedure with respect to grinding was the same as in Example I. The ore used was the same as that in Example I except that it had been subject to atmospheric oxidation in storage for up to 2 years. The ore pulp was conditioned in the flotation cell for about 1 minute with the collector and frother as indicated in Table IV. After 4 minutes of flotation, an additional

increment of 0.04 #/t. frother was added to the cell and flotation continued for a total of 9 minutes. No artificial sulfidization was used in the referenced tests. Table V shows the metallurgical results obtained.

TABLE IV

| Test No. | Collector                                                                                    | #/T   | Iso-propanol, #/T | Pine oil, #/T |
|----------|----------------------------------------------------------------------------------------------|-------|-------------------|---------------|
| 1.....   | Di-(N,N,N-trimethyl-N-tallowammonium) dithiocarbonate.                                       | 0.051 | 0.116             | 0.04          |
| 2.....   | N,N,N-trimethyl-N-tallowammonium sodium dithiocarbonate.                                     | 0.049 | 0.096             | 0.04          |
| 3.....   | Di-(N,N-dimethyl-N,N-ditallowammonium) dithiocarbonate.                                      | 0.052 | 0.097             | 0.04          |
| 4.....   | N,N-dimethyl-N,N-ditallow ammonium sodium dithiocarbonate.                                   | 0.056 | 0.088             | 0.04          |
| 5.....   | Di-(N,N-dimethyl-N,N-dicocoammonium) dithiocarbonate.                                        | 0.049 | 0.074             | 0.04          |
| 6.....   | N,N-dimethyl-N,N-dicoco ammonium sodium dithiocarbonate.                                     | 0.052 | 0.156             | 0.04          |
| 7.....   | Di-(N,N,N-trimethyl-N-cocoammonium) dithiocarbonate.                                         | 0.052 | 0.156             | 0.04          |
| 8.....   | N,N,N-trimethyl-N-coco ammonium sodium dithiocarbonate.                                      | 0.049 | 0.147             | 0.04          |
| 9.....   | N,N-dimethyl-N-coco-N',N',N'-trimethyl trimethylene di-ammonium di-(sodium dithiocarbonate). | 0.05  | 0.200             | 0.04          |

TABLE V

| Test No. | Analyses, weight percent Cu |       | Distribution, weight percent recovery of Cu in concentrate |
|----------|-----------------------------|-------|------------------------------------------------------------|
|          | Concentrate                 | Tails |                                                            |
| 1.....   | 27.85                       | 0.37  | 92.64                                                      |
| 2.....   | 21.27                       | 0.23  | 95.92                                                      |
| 3.....   | 22.01                       | 0.95  | 80.34                                                      |
| 4.....   | 24.49                       | 0.67  | 87.50                                                      |
| 5.....   | 22.19                       | 0.98  | 77.51                                                      |
| 6.....   | 23.93                       | 0.39  | 93.84                                                      |
| 7.....   | 26.59                       | 0.55  | 88.00                                                      |
| 8.....   | 22.42                       | 0.33  | 93.02                                                      |
| 9.....   | 21.25                       | 0.22  | 95.60                                                      |

#### EXAMPLE III

In each test a 500 gram sample of fresh unoxidized copper ore was ground for 2 minutes in a laboratory ball mill at 50% solids in a water suspension with 13 grams of CaO being added. The ground ore pulp was charged directly to a Fagergren cell for flotation, the pump was diluted to approximately 25% solids, pine oil as frother and the collector were added at the rates indicated in Table VI, and a one minute conditioning time was al-

lowed before the air was turned on. An additional increment of 0.04 #/t. of pine oil was added after 4 minutes float time and flotation continued for a total of 9 minutes. The pH was maintained at 12.0 to 12.3 with CaO. The collectors used were made up at various concentrations in isopropyl alcohol except in those tests where alcohol addition in Table VI is not noted, in which cases water solutions of the collector were used. Only the first rougher concentrate was collected. The results are shown in Table VII.

TABLE VI

| Test No. | Collector                                                | Collector, #/T | Iso-propanol, #/T | Pine oil, #/T |
|----------|----------------------------------------------------------|----------------|-------------------|---------------|
| 1.....   | Di-(N,N-dimethyl-N,N-dicocoammonium) dithiocarbonate.    | 0.133          | 0.200             | 0.08          |
| 2.....   | N,N-dimethyl-N,N-dicoco ammonium sodium dithiocarbonate. | 0.074          | 0.222             | 0.08          |
| 3.....   | Di-(N,N,N-trimethyl-N-cocoammonium) dithiocarbonate.     | 0.079          | 0.237             | 0.08          |
| 4.....   | N,N,N-trimethyl-N-coco ammonium sodium dithiocarbonate.  | 0.074          | 0.222             | 0.08          |
| 5.....   | do.....                                                  | 0.05           | .....             | 0.08          |
| 6.....   | Di-(N,N,N-trimethyl-N-cocoammonium) dithiocarbonate.     | 0.05           | .....             | 0.08          |

TABLE VII

| Test No. | Analyses, weight percent Cu |       | Distribution, weight percent recovery of Cu in concentrate |
|----------|-----------------------------|-------|------------------------------------------------------------|
|          | Rougher concentrate         | Tails |                                                            |
| 1-----   | 26.20                       | 0.18  | 96.49                                                      |
| 2-----   | 24.64                       | 0.18  | 96.64                                                      |
| 3-----   | 29.87                       | 0.37  | 92.42                                                      |
| 4-----   | 29.13                       | 0.26  | 94.76                                                      |
| 5-----   | 21.47                       | 0.17  | 96.50                                                      |
| 6-----   | 22.78                       | 0.32  | 93.28                                                      |

## EXAMPLE IV

This series of tests was carried on using the flotation procedure as described in Example III, the ore sample used being considered as severely oxidized due to an extended period of storage. The collector was added to the pulp in the amounts indicated in Table VIII, along with 0.04 #/t. pine oil. After 4 minutes of flotation, a second increment of 0.01 #/t. pine oil was added and flotation was continued for 5 minutes for a total of 9 minutes flotation time. The collectors were applied either as  $\frac{1}{2}\%$  or 1% water solutions, or as the undiluted chemical as synthesized. The latter existed at various strengths in isopropanol from synthesis procedures. The referenced tests were run without artificial sulfidation of the oxidized copper sulfide minerals with inorganic sulfur chemicals. Results were as set out in Table VIII.

wherein X is a monovalent cation selected from the group consisting of an alkali metal and a quaternary ammonium radical having the structure  $(R_1R_2R_3R_4N)^+$ , each  $R_1$ ,  $R_2$ ,  $R_3$  and  $R_4$  is selected from the group consisting of aliphatic hydrocarbon radicals having from 1 to 22 carbon atoms, provided that at least one and not more than 2 of the  $R_2$ ,  $R_3$  and  $R_4$  radicals contain from 6 to 22 carbon atoms; y is an integer from 1 to 2; and M is selected from the group consisting of  $R_1$  and  $-(CH_2)_xR_5R_6R_7NOCSS$  wherein each  $R_5$ ,  $R_6$  and  $R_7$  is selected from the group consisting of alkyl radicals having from 1 to 3 atoms and x is an integer from 2 to 4.

2. The process of claim 1 in which the ores are copper sulfide ores.
3. The process of claim 2 in which the copper sulfide ores are oxidized.
4. The process of claim 1 in which at least one of the  $R_2$ ,  $R_3$ , and  $R_4$  radicals contains at least 12 carbon atoms and X is sodium.
5. In a process for froth flotation separation of sulfide minerals from metallic sulfide ores, the step of conditioning a water suspension of finely-divided metallic sulfide ores with a dithiocarbonate, said dithiocarbonate being N,N,N-trimethyl-N-cocoammonium sodium dithiocarbonate.
6. The process of claim 5 in which said dithiocarbonate is di-(N,N,N-trimethyl-N-cocoammonium) dithiocarbonate.

TABLE VIII

| Test No. | Collector class                                           | Form of collector percent active in isopropanol or $H_2O$ | Collector #/T | #/T isopropanol added with collector | Weight percent Cu |       | Distribution, weight percent recovery of Cu in concentrate |
|----------|-----------------------------------------------------------|-----------------------------------------------------------|---------------|--------------------------------------|-------------------|-------|------------------------------------------------------------|
|          |                                                           |                                                           |               |                                      | Rougher           | Tails |                                                            |
| 1-----   | N,N,N-trimethyl-N-tallowammonium sodium dithiocarbonate.  | 33.5% in isoprop-----                                     | 0.0485        | 0.096                                | 21.27             | 0.23  | 95.92                                                      |
| 2-----   | do                                                        | 1/2% in $H_2O$ -----                                      | 0.05          | 0.099                                | 21.29             | 1.10  | 74.26                                                      |
| 3-----   | Di-(N,N,N-trimethyl-N-tallowammonium) dithiocarbonate.    | 30% in isoprop-----                                       | 0.051         | 0.116                                | 27.85             | 0.37  | 92.64                                                      |
| 4-----   | do                                                        | 1% in $H_2O$ -----                                        | 0.05          | 0.116                                | 22.44             | 0.31  | 93.28                                                      |
| 5-----   | N,N-dimethyl-N,N-ditallowammonium sodium dithiocarbonate. | 33% in isoprop-----                                       | 0.056         | 0.088                                | 24.49             | 0.67  | 87.50                                                      |
| 6-----   | Di-(N,N-dimethyl-N,N-ditallowammonium) dithiocarbonate.   | 33% in isoprop-----                                       | 0.052         | 0.097                                | 22.01             | 0.95  | 80.34                                                      |
| 7-----   | Di-(N,N-dimethyl-N,N-dicocoammonium) dithiocarbonate.     | 40% in isoprop-----                                       | 0.049         | 0.074                                | 22.19             | 0.98  | 77.51                                                      |
| 8-----   | N,N-dimethyl-N,N-dicocoammonium sodium dithiocarbonate.   | 25% in isoprop-----                                       | 0.052         | 0.156                                | 23.93             | 0.30  | 93.84                                                      |
| 9-----   | Di-(N,N,N-trimethyl-N-cocoammonium) dithiocarbonate.      | 25% in isoprop-----                                       | 0.052         | 0.166                                | 26.59             | 0.55  | 88.00                                                      |
| 10-----  | N,N,N-trimethyl-N-cocoammonium sodium dithiocarbonate.    | 25% in isoprop-----                                       | 0.049         | 0.147                                | 22.42             | 0.33  | 93.02                                                      |
| 11-----  | Di-dithiocarbonate from Duomeen C                         | 1% in $H_2O$ -----                                        | 0.05          | 0.200                                | 21.25             | 0.22  | 95.60                                                      |
| 12-----  | Std. Minerac 27                                           | 100% active-----                                          | 0.054         | -----                                | 7.42              | 2.08  | 29.30                                                      |

While in the foregoing specification, we have set forth specific process steps and collector compounds in considerable detail for the purpose of illustrating embodiments of the invention, those skilled in the art will appreciate that variations can be made without departing from the spirit and scope of the invention.

We claim:

1. In a process for froth flotation separation of sulfide minerals from metallic sulfide ores, the step of conditioning a water suspension of finely-divided metallic sulfide ores with a dithiocarbonate having the following structure:



50 7. The process of claim 5 in which said dithiocarbonate is N,N-dimethyl-N-coco-N',N',N'-trimethyl trimethylene di-ammonium di-(sodium dithiocarbonate).

## References Cited

## UNITED STATES PATENTS

- 55 1,902,317 3/1933 Wright ----- 209—166  
 FOREIGN PATENTS  
 126,816 5/1959 U.S.S.R.

60 FRANK W. LUTTER, Primary Examiner.

R. HALPER, Assistant Examiner.